

Patented Feb. 1, 1927.

## UNITED STATES PATENT OFFICE.

FRIEDRICH W. WEBER, OF HACKENSACK, NEW JERSEY.

## MINERAL-TANNED LEATHER AND METHOD OF MAKING THE SAME.

No Drawing.

Application filed March 19, 1925. Serial No. 16,860.

This invention relates to leather and it particularly relates to leather tanned with metal oxides of the general type  $Me_2O_3$ , preferably such as iron oxide, chromium oxide and the like and with the oxides of the rare earth metals, or compounds, very poor in acid, of the same, the object of the invention being to provide means by which a leather of superior qualities can be obtained at a low 10 price and in a short time.

The tanning properties of iron oxide have been known for several centuries but the difficulty to find a proper solution of this oxide allowing its convenient application in 15 the tanning process was too great as to favor a development of the iron tanning process notwithstanding the well-known efforts by Knapp and his many successors.

The difficulties in the application of the 20 salts of the various metals are surprisingly solved and the tanning greatly simplified by my new invention of combining the tanning effected by iron and chromium salts and those of metals closely related to iron and 25 chromium, with my new tanning method of applying the salts of the rare earth metals as described in my copending patent application, entitled "Treating animal tissue", filed under Serial No. 704,282. The metals 30 of the iron group are preferably applied in my new process in the form of their chlorides or sulfates, their application depending to a large extent on the price as to which gives the greatest economic advantages.

35 My new invention is based on the saturation of pickled hides with a solution of basic acetates of the rare earth metals before they come in touch with a tanning solution consisting of one of the salts of the metals referred to above, for instance with my new colloidal ferric chloride solution made as described below, and to dry the hides thus saturated. During this drying process acetic acid is split off and vaporized causing a 40 deposition of oxides of the rare earth metals, or of more basic compounds of the same which are very poor in acid, within the hide whereby a leather is obtained similar to that furnished by tanning with alum and salt, but 45 having a greater quantity of metal oxide in view of the higher atomic weight of the rare earth metals. The dried hides, or leather, are returned to the same bath of basic acetates of the rare earth metals, the bath having 50 a content of sodium chloride corresponding to 5° Bé. and containing for each liter

of its volume 100 cc. of a saturated solution of acetates of the rare earth metals.

To this bath I now add the colloidal basic ferric chloride solution referred to above. 60 Adding this ferric chloride solution causes no precipitation whatever, on the contrary the tanning process sets in immediately, thin hides being tanned in about two hours, while thicker ones require a correspondingly longer time. The tanning effect produced hereby is so perfect that the hides can be removed immediately from the tanning bath to the drying chamber and ultimately, when dry, show no shrinking whatever, nor are there any hard spots, nor any rubberlike swelling, they can immediately be worked mechanically by stretching and staking. 70 If these leathers are soaked in water their content of sodium chloride is leached 75 cut as well as a very minute quantity of rare earth metals, but not a trace of iron.

The unwashed, dried hide, or leather, is then treated in a substantially neutral soap solution at a temperature of 40-50° C., dried 80 again and the treatment with soap is then repeated. This treatment renders the leather strong, shiny on the surface and water repellent to a remarkable degree.

85 After the tanning process is finished, the iron is quantitatively precipitated from the tanning bath as basic ferric acetate and only a little sodium carbonate needs to be added to the supernatant, almost colorless solution to quantitatively precipitate the carbonates 90 of the rare earth metals, free of iron, the filtrate from the carbonates containing all sodium chloride and a little acetate. This sodium chloride solution will probably have a concentration of 5° Bé. as very little dilution takes place during the tanning process, otherwise it can be adjusted to this concentration and be used over again in the tanning process.

95 Why it is possible that a good tanning effect can be obtained with the process without a premature precipitation of the iron liquor, appears to be explained by my observation that the presence of the basic acetates of the rare earth metals precipitate the iron oxide only very gradually and that upon the addition of this iron liquor to the solution of the acetates of the rare earth metals even in the presence of sodium chloride a clear purple-red solution is formed, 100 which gradually turns smoky so slowly that sodium chloride can be applied without any 105

difficulty whatever for preventing the hides from swelling.

Example for preparing the colloidal ferric chloride solution:

- 5 I apply the crystallized ferric chloride containing 12 mol of water, corresponding approximately to a 50%  $\text{Fe}_2\text{Cl}_6$ . Then I dissolve 1 lb. ferric chloride in 1 lb. water and dilute to 1 liter. I thus obtain a solution of 10  $25^\circ \text{Bé} = 1.21$  spec. gr. = 42 Twaddell = 25%  $\text{Fe}_2\text{Cl}_6$  solution.

To 200 cc. of this solution are added preferably 25 grams of a 57% mixture of carbonates of the rare earth metals (computed 15 on oxide) which must not necessarily be absolutely free of phosphate, or sulfate, and with a copious discharge of gases according to the equations



in which Fe stands as representative of any 25 metal of the iron group forming oxides of the general type  $\text{Me}_2\text{O}_3$  and lanthanum, the carbonate of which can be safely considered constituted as stated above, represents any 30 of the rare earth metals, a dark-red, transparent and clear solution is obtained; it thickens within a few hours into a rather viscous syrup which dissolves in water in every proportion and even on boiling stays clear; it may turn smoky at continued heating, but the solution always clears again on cooling. If one adds, however a single kernel of sodium sulfate to the clear solution either before or after boiling, immediately a heavy precipitation of ferric 35 hydrate takes place while the rare earth metals stay dissolved.

This effect of the sodium sulfate causes a 40 coagulation, or precipitation, of ferric-oxyhydrate; if this precipitate happens to the solution always turns more acid the more ferric-oxyhydrate is precipitated; this acid, however, cannot do any harm to the hides, nor will it re-dissolve the ferric-oxyhydrate precipitated in the hide about to be tanned; it is obvious that the salts of the rare earth 45 metals, still present in the tanning liquor, then continue the tanning process and cover the iron already deposited in the leather.

To facilitate the understanding of my invention I shall describe by way of example 50 how I proceed to carry the same into effect:

Dry calf hides for instance, which were previously pickled in the usual bath containing 1% sulphuric acid and 5% sodium chloride 55 are soaked in a sodium chloride solution of 5°  $\text{Bé}$ . until they are thoroughly penetrated and free of folds and show a uniform appearance. As soon as this stage is reached I add to this bath for each liter of its volume 60 100 cc. of a saturated solution of basic

acetates of the rare earth metals which may be bought in the market in the form of a 16% solution computed on rare earth metal oxide. In this sodium chloride acetate solution the hides are well agitated for 3-5 70 hours, are then taken out and suspended so as to drain all liquid back into the bath, whereupon the hides are dried at a moderate temperature. It is well to effect this drying over night; during this drying process acetic acid is split off and vaporized and the more basic acetates of the rare earth metals are well fixed upon the hides, but they should not be dried too much so as to assume a great stiffness. The hides are then returned 75 to the same bath to which I then add all at once 50 cc. of above colloidal ferric chloride solution, deacidified as explained above with the carbonates of the rare earth metals, for each 1 liter of bath liquor, without causing 80 a precipitation in the solution even in the presence of sodium chloride and without swelling the hides, an excellent tanning effect 85 takes place immediately. As soon as this tanning process has proceeded so far that 90 the hides are tanned also at their thick parts, the hides are taken out of the bath, drained off the excess of liquor and then dried which does not require the usual nailing as they 95 will not shrink and reduce in their surface, nor will they get horny during the drying process.

It is noteworthy that the unwashed dry leather obtained by my new process does not 100 show the dangerous efflorescence of sodium chloride so often noticed in the products of other mineral tanning processes. From practical considerations it appears desirable to dry with the sodium chloride in the leather and to submit the same then to the 105 soaping process without washing the leather previous to this soaping process, as the leather thereby gets denser and water-repellent to a high degree.

Inasmuch as the leather was first saturated 110 in the tanning process with the basic acetates of a mixture of the rare earth metals, the oxides of which are therefore fixed during the drying process on the fibers of the hides, and was subsequently treated with the 115 colloidal ferric chloride solution containing simultaneously also the basic chlorides of the rare earth metals, the iron oxide, or any other oxide of the general  $\text{Me}_2\text{O}_3$ , is fixed upon the fibers of the hides together with 120 the oxides of the rare earth metals; it can therefore safely be said in view of the foundation laid by the preliminary treatment of the hides with the acetates of the rare earth metals and the tanning action by the basic 125 chlorides of the rare earth metals simultaneously with the precipitation of the iron as ferric-oxyhydrate, that the iron oxide is thoroughly intermixed with the oxides of the rare earth metals and is encased by the same 130

owing to the deposit of the oxides of the rare earth metals after nearly all iron oxide has been precipitated out of the colloidal tanning liquor. Though the iron oxide as well as the oxides of the rare earth metals deposited in the leather are generally insoluble in water, their relation to the hide-substance, during the very short time that the tanning process is going on, is such that at least part of all the various oxides enter into a reaction with any soap solution with which the treated hide may be brought into contact, thereby forming the respective soaps; whether this is due to the influence of hydroxyl-groups still present in the molecules of the oxides or due to traces of acid having just segregated from the basic salts in the tanning process and still present in the hide-substance, is difficult to say.

The obtained leather exhibits a pleasant light tan color which logically seems to be the result of the double tanning process by means of iron and the rare earth metals; it is free of the dark-red color of the other so-called iron-leathers which excludes a dyeing with light shades.

From the aforesaid description it is evident that the leather during the tanning process was never touched by sulfuric acid, but only by tanning solutions of weak acid reaction, among them one with a volatile organic acid, wherefore a dangerous concentration of acid cannot take place in the finished leather; moreover, the presence of the oxides of the rare earth metals prevents the ferric oxide from being reduced to ferrous oxide at the expense of the hide itself and causes, if traces of hydrochloric acid should be split off, to have them immediately neutralized.

To the above statements that the tanning liquor of the acetates of the rare earth metals containing also the colloidal ferric chloride solution deacidified as described above with the carbonates of the rare earth metals after the precipitation and filtration of the basic iron acetate yields a clear solution and that the carbonates of the rare earth metals may be precipitated therefrom by sodium carbonate I wish to add that these regenerated carbonates are of much greater purity than they were when first applied, since the last traces of iron of the rare earth metals have been precipitated with the whole mass of iron; this iron free solution of the regenerated earth metals may of course also be used over again in the tanning process to save their precipitation as carbonates.

The well known difficulties in the application of chromium alum as a tanning material are soon overcome by extending my new process also to this material. I have now found a way of producing an excellent tanning solution by starting directly from chromium alum, and that the new tanning

solution thus obtained has not only an excellent power of penetrating the animal hide without reducing the hide in surface, but also tans it completely in a very short time. Moreover, the tanning liquor stays clear until the tanning process is finished and thus offers the possibility to let the hide soak over night in the bath without any danger of forming undesirable spots, or that the hides swell, or take on too much acid, and thus the application of chromium alum is rendered possible by my new and improved process, which I am going to describe below, though the chromium alum contains only the same amount of chromium as the sodium bichromate (M. W. 300) which has only one third of the molecular weight of that of the chromium alum.

For the better understanding of my new process I will give an example of how I make my new tanning solution from chromium alum:

200 grams crystallized chromium alum are dissolved in 500 gr. water and boiled until a dark green solution is formed; to this solution I add then a paste of water and 40 grams of carbonates (containing 57% oxides) of the rare earth metals, and with the discharge of gas not only a reduction in the sulfuric acid content of the alum is obtained, but also a solution of a basic chromium sulfate and of basic sulfates of the mixed rare earth metals. During this reaction some chromium oxyhydrate is precipitated together with some calcium sulfate as the carbonates of the rare earth metals are liable to contain some lime, and also iron which accompanies the rare earth metals as well as the chromium alum. The solution thus obtained is diluted up to 1 liter, hereafter it is allowed to stand to settle and the clear solution is then ready for use.

In the case of chrome tanning I recommend the application of the carbonates of the rare earth metals particularly for the deacidification of all alums suitable for tanning. In explanation of this situation I beg to refer to the observation of many authorities in the chemistry of tanning, who state that the well dissociated or green chromium solutions display the greatest tanning effect. If now to chromium alum, which contains the potassium sulfate as unnecessary ballast, the carbonates of the rare earth metals are added for the purpose of neutralizing the sulfuric acid as well as for the purpose of forming salts having tanning properties, the latter find in the potassium sulfate an agent to which they have a great affinity.

It is known that the soluble sulfates of the rare earth metals, insoluble in concentrated potassium or sodium sulfate solutions, may be precipitated by the said solutions from the solutions of the chlorides

or sulfates of the same, which speaks for their great affinity to potassium or sodium sulfate. In the case of my new tanning solution we find such double sulfates in soluble form together with the well dissociated basic chromium sulfate; this fact explains their eminent tanning power without being too acid or too basic. The tanning effect accomplished by this solution is also 10 favorably influenced by the slightly slower action of the double sulfates of the rare earth metals, and yet the tanning takes place so surprisingly quick; in this connection I want to mention that by washing the tanned 15 hides only the mechanically adhering part of the tanning solution is removed, whereas that part, which penetrates the hide, is hydrolyzed which explains that the hides, originally appearing green, immediately assume 20 a lighter color and give off the acid when washed with water. The hides treated with this new tanning solution are finally washed with water until they turn neutral litmus paper faintly red and the water itself stays 25 neutral. Now the hides can be soaped.

This soaping process is carried out as follows: I prepare from a good neutral textile soap, which has 10% fixed alkali and 30% water and does not contain more than 0.1% 30 free alkali, a 5% solution and work the hides therein at a temperature of substantially 60° C. until they are thoroughly saturated with soap solution and show a sufficiently neutral reaction. Owing to the formation of chromium-soap, covered with the practically absolutely insoluble soap of these rare earth metals, a very soft leather of velvet or cloth like feeling is obtained, which is dried and subsequently may be fat liquored 35 as desired. I want to emphasize that it is of advantage to introduce the well washed hides into the soap solution when still showing a slightly acid reaction for the reason that any soap, originally absolutely neutral, 40 splits off some alkali which then meets in the leather with some traces of acid and is thus easily neutralized.

By my efforts to overcome the above described shortcomings peculiar to the Schultz 50 process I have found out that a solution, obtained in the manufacture of rare earth metal compounds, may be applied with great advantage.

When in the manufacture of thorium salts the chlorides of the rare earth metals, obtained by fusing monazite sand with alkali and dissolving the washed oxides in hydrochloric acid in a form free of phosphates, are acted upon with a solution of sodium thiosulfate with the intention to separate the thorium in the form of its thiosulfate, the solution of the chlorides obtained after filtering off the thorium thiosulfate and the molecular sulfur, contains a great excess of 55 sodium thiosulfate which is necessary if the

thorium is to be precipitated quantitatively. This chloride solution now contains the chlorides of the remaining rare earth metals with very little iron and as it is neutral, it is for various reasons extremely suitable 71 as a reduction bath for a two bath process. For the first it contains enough sodium thiosulfate to reduce all chromic acid, which was fixed upon the hides in the first bath, and secondly it contains a sufficient quantity 76 of the chlorides of the rare earth metals which immediately act upon the hide impregnated with chromic acid as soon as it is introduced into the bath simultaneously with the reducing action of the thiosulfate 80 generating basic chromium chloride which acts as a tanning agent and is supported in its action by the chlorides of the rare earth metals without the necessity of adding any great amount of acid, which is important 85 because this fact reduces the precipitation of molecular sulfur very considerably; this molecular sulfur is furthermore covered by the oxides of the rare earth metals which protect it against further oxidation. The 90 whole tanning process is complete, and the leather shows very seldom any swelling and has a better feeling than with the well known Schultz chrome tanning process; they are also more easily finished by any of the 95 well known ways. I may say that empty spots, so often encountered in the Schultz process are avoided because the presence of the rare earth metals appears to avoid such spots even if slight bleeding should take 100 place as with the Schultz process. This does not exclude that in the reduction bath chlorides of the rare earth metals may be directly applied after a sufficient amount of thiosulfate has been added thereto.

It stands to reason that I do not restrict myself to chromium alum as a source for a tanning solution, but I just as well start from the sodium bichromate which I reduce in the manner described by U. S. Patent 110 1,221,929, issued to me on April 10, 1917. According to this patent I effect the reduction by acidulating the sodium bichromate solution and then adding a substance liberating SO<sub>2</sub>, for instance sodium bisulfite to 115 the same; the solution of chromium sulfate obtained thereby may then be deacidified by the carbonates of the rare earth metals that the acid combines with the same forming thereby basic sulfates of the rare earth metals, as already described above.

I have furthermore found that I may proceed in the following manner especially if it is intended to produce a chrome leather of velvet like, soft feeling which is especially characterized by a smooth grain side:

The hides are treated in a 5° Bé. sodium chloride solution, to which bath, while being agitated, for each liter of its volume 100 cc. of a basic acetate solution of the rare earth 120

metals are added. In this mixture of solutions the hides are well agitated for about 3 hours, then they are taken out of the bath, drained off, and put up for drying over 5 night, whereby the oxides of the rare earth metals are completely fixed upon the hides. The hides thus dried are then put back into the same bath to which I add for each liter of its volume 100 cc. of a neutral chromium 10 solution, for instance of a chromium alum deacidified as described above. Here it can be observed that the tanning solution does not only stay clear, but gradually turns violet because of the formation of the sulfates of the rare earth metals. The tanning 15 of the hides progresses continuously; after three hours they are taken out of the bath. This operation can also be performed in one bath by adding to the sodium-chloride solution 20 for each liter of its volume, according to the thickness of the hide, 25 cc. of a basic acetate solution of the rare earth metals and of a corresponding quantity of chromium alum deacidified as described above; 25 eventually the sodium chloride may be substituted by sodium sulfate. This modified procedure extends the time of the tanning process quite considerably, but I obtain a soft and white leather. The leather may 30 finally be washed and soaped which yields a snow-white and very durable leather.

In order to obtain a chrome leather of light shade I can modify aforesaid process in the following manner:

35 I deacidify aluminum sulfate, or potassium alum, sodium alum or any other suitable alum salt in a concentrated solution; for instance I dissolve 190 grams potassium aluminum sulfate in 500 cc. of water and 40 add thereto 40 gr. carbonates of the rare earth metals until at an elevated temperature a lasting precipitate is formed whereby iron hydrate calcium sulfate and other impurities of the rare earth metals are precipitated; I dilute the solution thus obtained to 45 1 liter and allow to stand to clarify; 100 cc. of the clear solution and 100 cc. of the neutralized chromium alum are then added to each liter of the bath volume and the hides 50 then tanned therein to be subsequently washed and soaped. All the leathers thus obtained are of course fat liquored in any of the well known ways but inasmuch as these after treatments are not part of the 55 real tanning process, this branch of the treatment of leather is here not dwelled upon.

It is also possible to obtain special effects 60 by treating the leather with egg-yolk and wheat-flour, but also these methods are here not further referred to as it is my intention to demonstrate by this description how by the methods based upon the application of the rare earth metals compounds the various 65 processes of tanning, especially those by iron

and chromium salts, and by salts of the metals more or less related to aforesaid metals, can be improved and simplified, as one always works with clear solutions of excellent tanning power as their basicity is just right 70 and is governed by a very fortunate proportion between the high atomic weight of the rare earth metals and the relatively low amount of acid, i. e. in other words the rare earth metals have in their salts, whether sulfates, or chlorides, compared with the corresponding salts of Al, Cr, Fe, Mn, etc. the lowest amount of acid in their molecule; furthermore it is due to the insolubility of 75 the soaps of the rare earth metals that the 80 leather obtained by the above processes are full and of soft feeling.

In recent years the lactic acid has been introduced into tanning; though lactic acid has proved as an excellent material for the 85 deliming of the hides, it could only be used in the form of its alkalia metal salts as a reducing agent; for if lactic acid comes into contact with hides impregnated with chromic acid, it is oxidized to formaldehyde and 90 acetic acid. I have found out that the lactates of the rare earth metals may well be applied as a reducing agent in a reduction bath where they are transferred into the acetates thus offering a way for applying 95 lactic acid with greater advantage for tanning purposes.

What I claim is:

1. The method of tanning hides, comprising soaking pickled hides in a sodium chloride solution, adding thereto the solution of a rare earth metal compound capable of forming basic salts, agitating the hides in the mixture of the aforesaid salt solutions, drying the hides thus treated, returning the 100 dried hides to aforesaid mixtures of salt solutions, adding to said mixture a solution containing the reaction mixture of a salt of a metal, forming an oxide of the type  $Me_2O_3$ , with a basic compound of the rare 105 earth metals, and drying the hides thus treated.

2. The method of tanning hides, comprising soaking pickled hides in a sodium chloride solution, adding thereto the solution of a rare earth metal compound capable of forming basic salts, agitating the hides in the mixture of the aforesaid salt solutions, drying the hides thus treated, returning the 115 dried hides to aforesaid mixtures of salt solutions, adding to said mixture the solution containing the reaction mixture of a salt of a metal, forming an oxide of the general type  $Me_2O_3$ , with a carbonate of the rare earth metals, and drying the hides thus treated.

3. The method of tanning hides with metal salts, said method comprising acting upon a hide with a solution containing a reaction mixture of a salt of a metal, forming 120

130

an oxide of the type  $Me_2O_3$ , with a basic compound of a rare earth metal.

4. The method of tanning hides with metal salts, said method comprising acting upon a hide with a solution containing a reaction mixture of a salt of a metal, forming an oxide of the type  $Me_2O_3$ , with a carbonate of a rare earth metal.

5. The method of tanning hides, comprising soaking the pickled hides in a sodium chloride solution, adding to aforesaid bath of sodium chloride the solution of a salt of the rare earth metals capable of forming basic salts, agitating the hides in the mixture of the aforesaid salt solutions, drying the hides thus treated, returning the dried hides to the aforesaid mixture of salt solutions, adding to said mixture a solution containing the reaction mixture of a chromium alum with a basic compound of the rare earth metals, and drying the hides thus treated.

6. The method of tanning hides, comprising soaking the pickled hides in a sodium chloride solution, adding to aforesaid solution of sodium chloride the solution of an acetate of one of the rare earth metals, agitating the hides in the mixture of the aforesaid two salt solutions, drying the hides thus treated, returning the dried hides to aforesaid mixture of salt solutions, adding to said mixture a solution containing the reaction mixture of a chromium alum with a basic compound of the rare earth metals, and drying the hides thus treated.

7. The method of tanning hides, comprising soaking the pickled hides in a sodium chloride solution, adding to aforesaid solution of sodium chloride the solution of basic acetates of the earth metals, agitating the hides thus treated in the mixture of aforesaid two salt solutions, drying the hides thus treated, returning the dried hides to the aforesaid mixture, adding to said mixture a solution containing the reaction mixture of a chromium alum with a carbonate of the rare earth metals, and drying the hides thus treated.

8. The method of tanning hides, comprising soaking the pickled hides in a sodium chloride solution, adding to aforesaid solution of sodium chloride the solution of an acetate of one of the rare earth metals, agitating the hides in the mixture of the aforesaid two solutions, drying the hides thus treated, returning the dried hides to the aforesaid mixture of salt solutions, adding to said mixture a solution containing the reaction mixture of a chromium alum with a basic compound of the rare earth metals, drying the hides thus treated, and soaking the dry hides in a soap solution.

9. The method of tanning hides, comprising soaking the pickled hides in a sodium chloride solution, adding to aforesaid solu-

tion of sodium chloride the solution of basic acetates of the rare earth metals, agitating the hides thus treated in the mixture of aforesaid two salt solutions, drying the hides thus treated, returning the dried hides to the aforesaid mixture, adding to the said mixture a solution containing a reaction mixture of a salt of a metal forming an oxide of the type  $Me_2O_3$  with a carbonate of the rare earth metals, drying the hides thus treated, and soaking the dry hides in a soap solution.

10. The method of tanning hides, comprising acting upon a solution of a chromium salt with a substance capable of acting upon aforesaid chromium salt thereby forming per se a salt capable of tanning hide and simultaneously a basic chromium salt, and acting with the solution thus obtained upon the hides.

11. The method of tanning hides, comprising heating the solution of a chromium alum at substantially its boiling point until said solution turns green, adding to aforesaid solution a basic compound of the rare earth metals thereby forming basic sulfates of the rare earth metals and basic chromium sulfate, and acting with the solution thus obtained upon the hides.

12. The method of tanning hides, comprising heating the solution of a chromium alum at substantially its boiling point until said solution turns green, adding to aforesaid solution the carbonate of a rare earth metal thereby forming a basic sulfate of the rare earth metals, and acting with the solution thus obtained upon the hides.

13. The method of tanning hides, consisting in acting upon a solution containing a salt containing aluminum sulfate with a carbonate of the rare earth metals, combining the solution thus obtained with a solution obtained by acting upon chromium alum with a carbonate of the rare earth metals, adding the aforesaid combined solutions to a bath of sodium chloride, acting with the mixture of all three solutions upon the hides, washing the hides thus treated, and acting upon the washed hides with a soap solution.

14. As a new article of manufacture, a double tanned leather having fixed upon its fibers a deposit of one of the oxides of the rare earth metals and upon aforesaid deposit another one consisting of a mixture of a chromium-oxide and of an oxide of a rare earth metal.

15. As a new article of manufacture, a double tanned leather having fixed upon its fibers a mixture of a metal oxide of the general type  $Me_2O_3$  and of an oxide of a rare earth metal.

16. As a new article of manufacture, a tanned leather having fixed upon its fibers a mixture of oxides consisting of those of chromium and of a rare earth metal.

17. As a new article of manufacture, a tanned leather having fixed upon its fibers tanned leather having fixed upon its fibers a mixture of oxides of aluminum, chromium and <sup>10</sup> of a mixture of oxides, consisting of that of rare earth metal. chromium and of a rare earth metal, and of In testimony whereof I hereunto affix my 5 a mixture of soap, consisting of that of signature. chromium and of a rare earth metal.

18. As a new article of manufacture, a

FRIEDRICH W. WEBER.